

B. McCOLLUM.

HYSTERESIS STARTING DEVICE FOR INDUCTION MOTORS.

APPLICATION FILED DEC. 12, 1911.

1,031,802.

Patented July 9, 1912.



Burton McCollum.

Inventor

Witnesses

Minnie Lester  
James W. Kelly

# UNITED STATES PATENT OFFICE.

BURTON McCOLLUM, OF WASHINGTON, DISTRICT OF COLUMBIA.

## HYSTERESIS STARTING DEVICE FOR INDUCTION-MOTORS.

1,031,802.

Specification of Letters Patent.

Patented July 9, 1912.

Application filed December 12, 1911. Serial No. 665,383.

To all whom it may concern:

Be it known that I, BURTON McCOLLUM, a citizen of the United States, and a resident of Washington, District of Columbia, have 5 invented a new and useful Hysteresis Starting Device for Induction-Motors, of which the following is a specification.

It is well known that alternating current induction motors, in order to have good 10 starting characteristics, should have a high resistance in the secondary circuit, while to have good running constants the secondary resistance should be low.

My invention has for its object to produce 15 a motor without mechanical complications of any kind in which the apparent resistance of the secondary circuit shall automatically vary so as to have a very low value at near full load speeds, and gradually increase with 20 decreasing speed to a relatively high value at standstill, thus enabling the motor to operate most satisfactorily under both starting and running conditions.

My invention applies particularly to the 25 type of motor having a rotor known as the squirrel cage rotor, and consists essentially in surrounding the short circuiting rings of the squirrel cage with auxiliary rings herein-after called hysteresis rings composed of a 30 magnetic material having certain characteristics specified below.

It is well known that when an electric circuit carrying an alternating current links with a magnetic circuit there will be a dissipation of energy in the magnetic material 35 which gives rise to an apparent increase in the resistance of the electric circuit, which increase of resistance can be expressed approximately by the formula

$$40 \quad R = \frac{nvB^{1.6}}{I^2},$$

where R is the increase of resistance, commonly called hysteresis resistance, f the frequency of the alternating current, B the maximum flux density reached by the magnetic material each cycle, I the current flowing in the electric circuit, n and v the hysteresis constant and volume respectively, of 50 the magnetic material. It will be seen from this equation that the increase in resistance tends to increase with increasing frequency, and since the frequency of the secondary currents in the short circuiting rings of the 55 squirrel cage is very low at high speed and relatively high at starting, it follows that

the hysteresis resistance will tend to be high at starting and low under running conditions. Further, in order that a sufficiently large resistance may be had to give the required starting torque without using too large a volume of magnetic material, it is desirable that the material used should have a high hysteresis constant. These conditions alone are, however, not sufficient to insure a 60 satisfactory rise in resistance with decreasing speed. It is well known that the current flowing in the short circuiting rings of the squirrel cage rotor increases greatly under ordinary conditions with decreasing speed, 65 and since the factor  $I^2$  appears in the denominator of the equation for hysteresis resistance, this tends to cause a decreasing resistance with decreasing speed, and if B remains practically constant, which is sub- 70 stantially the case provided the normal full load currents in the short circuiting rings are sufficient to magnetize the hysteresis rings practically to saturation, the increase 75 in  $I^2$  may more than counterbalance the in- 80 crease in  $f$  and thus cause an actual lowering of resistance with decreasing speed. In order to overcome this difficulty, it is necessary to so design the hysteresis rings that the factor B in the equation will greatly in- 85 crease with increasing current. In order to do this it is necessary to make the hysteresis rings of a material of such nature and of such proportions that the normal full load currents in the rotor will magnetize them 90 but feebly, but so that the starting currents will magnetize them to a relatively high value. Since, with every magnetic material, the permeability tends to rise at a certain critical value of magnetizing force, it is pos- 95 sible by selecting a material of a proper nature to make the factor B increase more rapidly than I throughout the range from full load to standstill, and in this way a large increase in resistance may be secured. 100 Since the normal load currents in the short circuiting rings of the squirrel cage are necessarily very large ordinary magnetic materials cannot be used for the hysteresis rings because they would be magnetized to a 105 degree approaching or reaching saturation by the full load currents of the motor. It is necessary to use materials having a relatively low permeability and the larger the normal currents in the rings, the lower the 110 permeability should be. It is important, however, not to make the permeability too

low since in this case the value of  $B$  would be too small even at starting and a very large volume of material would be necessary to secure the desired increase in resistance.

5 Best results are obtained when the hysteresis rings are so designed that the starting currents will magnetize them to a degree just approaching saturation, while the full load currents magnetize them to a degree far below this point. I have found that pure metals cannot be used for the hysteresis rings because the magnetic metals in their pure state have too high a permeability.

10 Numerous alloys of metals, however, and particularly those alloys containing manganese, when properly designed, give the desired results. Of these, I have found that an alloy of iron and manganese is most suitable, it being adapted for use in motors of

15 any size. It is characteristic of this alloy that by varying the proportion of manganese from zero to approximately twelve percent, any desired permeability from the maximum of pure iron to practically unity can be obtained, and at the same time, a high hysteresis constant is secured.

My invention is further described below, reference being made to the accompanying drawings.

30 Of the drawings: Figure 1 is an end elevation of the rotor to which my invention applies. Fig. 2 shows a modified construction of the hysteresis rings. Fig. 3 is a sectional view of a portion of the rotor including one of the short circuiting rings.

35 Referring to Fig. 1, 1 is the laminated core which may be of the usual type, 2 the conductors of the squirrel cage winding, 3 the short circuiting ring, and 4 the hysteresis rings of magnetic material, which latter constitute the essential feature of my invention. It will be seen that between each pair of bars 2 there is placed a hysteresis ring 4 surrounding the short circuiting ring 3. When the alternating current flows in the short circuiting ring, alternations of magnetism are produced in the ring 4 which give rise to the hysteresis resistance mentioned above. The relation of the hysteresis rings 4 to the other parts of the structure is more clearly seen by reference to Fig. 3 which shows a section through the ring 3, a portion of one of the conductor bars 2, and the laminated core 1.

55 In some cases, especially in large motors where the hysteresis rings 4 are large, eddy currents induced therein may give rise to unequal distribution of magnetism which may be objectionable, and this can be avoided by the structure shown in Fig. 2. Here 4' shows the hysteresis rings made up of a number of thin sheets, which are effective in eliminating trouble from this source.

60 65 In putting the hysteresis rings 4 on the

short circuiting ring 3, the ring 3 is cut open and spread slightly at one point while the rings 4 are being put on, after which the ring 3 is closed by soldering, welding, or by other suitable means. The rings 4 are then uniformly spaced and the ring 3 connected to the bars 2 as shown in Fig. 1. Connection of the ring 3 to the bars 2 may be accomplished by soldering as shown, or by screws, bolts, or other suitable means.

70 It is obvious that the hysteresis rings hereinabove described can be used on either or both of the short circuiting rings of the squirrel cage, and may be grouped on either ring in any desired manner without departing from the generic principle of my invention.

75 I claim:

1. In an induction motor with squirrel cage rotor, short circuiting rings connected to the bars of the squirrel cage, rings of magnetic material surrounding said short circuiting rings, said magnetic rings being composed of a material having a high hysteresis constant, and being of such composition and so proportioned as to be magnetized to a high density by the starting currents in the short circuiting rings, but magnetized to a relatively low density by the normal full load currents.

80 85 90 95 100 105 110 115 120 125 130 135

2. In an induction motor with squirrel cage rotor, short circuiting rings connected to the bars of the squirrel cage, rings of magnetic material surrounding said short circuiting rings, said magnetic rings being composed of a material having a high hysteresis constant, and being of such composition and so proportioned as to have a high hysteresis resistance at low speeds of the motor, and a much lower hysteresis resistance at high speeds of the motor.

3. In an induction motor with squirrel cage rotor, short circuiting rings connected to the bars of the squirrel cage, rings of magnetic material surrounding said short circuiting rings, said magnetic rings being of such composition and so proportioned as to have a higher permeability when subjected to the magnetizing force due to the starting currents than when subjected to the magnetizing force of the normal full load currents in the short circuiting rings.

110 115 120 125 130 135

4. In an induction motor with squirrel cage rotor, short circuiting rings connected to the bars of the squirrel cage, rings of material surrounding said short circuiting rings, said magnetic rings being of laminated structure substantially as shown, and being of such composition and so proportioned as to have a higher permeability when subjected to the magnetizing force due to the starting currents than when subjected to the magnetizing force of the normal full load currents in the short circuiting rings.

5. In an induction motor with squirrel cage rotor, short circuiting rings connected to the bars of the squirrel cage, said short circuiting rings being surrounded by rings composed of a magnetic alloy of manganese. 5
6. In an induction motor with squirrel cage rotor, short circuiting rings connected to the bars of the squirrel cage, said short circuiting rings being surrounded by rings composed of an alloy of iron and manganese. 10
- BURTON McCOLLUM.

## Witnesses:

MINNIE LESTER,  
JESSIE C. McCOLLUM.